# EUROPEAN PATENT SPECIFICATION

(11) **EP 0 708 904 B1**
(45) Date of publication and mention of the grant of the patent: **05.02.2003**
(21) Application number: 95916918.6
(22) Date of filing: 10.04.1995
(51) Int. Cl.: F26B 3/00

(54) **Apparatus and method for drying charged battery plates**
Vorrichtung und Verfahren zum Trocknen von geladenen Batterieplatten
Appareil et procédé pour sécher des plaques d'accumulateur chargées

(30) Priority: 11.04.1994 US 225760
(43) Date of publication of application: 01.05.1996
(73) Proprietor: Tiegel, Ralph, G., Redwood City, CA 94062 (US)
(72) Inventor: TIEGEL, Ralph, G., Redwood City, CA 94062 (US); WEGNER, Paul, C., San Carlos, CA 94070 (US)
(74) Representative: Ebner von Eschenbach, Jennifer
(86) International application number: US9503936
(87) International publication number: WO95027878

(56) References cited:
- US-A- 2 484 527
- US-A- 2 732 631
- US-A- 3 413 728
- US-A- 4 099 337
- US-A- 5 040 974

## Description

### TECHNICAL FIELD

This invention relates to an apparatus and a method for drying charged battery plates comprising the features of the preamble of claim 1, respectively the preamble of claim 22. Such an apparatus is disclosed in US-A-3,413,728. Prior art figures 1, 2, and 3 illustrate this machine and the method of using it. With reference to those drawings and the specification of that patent it will be noted that in operation the door **13** is opened and a basket **20** containing battery plate groups is lowered into a drying chamber **18**. When closed, the door **13** relies upon a gasket around its periphery to maintain a seal.

A centrifugal fan **41** receives hot combusted gases from a combustion chamber **38** and mixes it with intake air which it then blows down the sloping surface in the direction the arrows shown over the charged plates. The hot air passes through the basket and thence through a support means **19,** and through a baffle means **28** and into a cooling chamber **25.** Within this cooling chamber a spray nozzle **27** sprays water into the air. The baffle **28** is designed to prevent the mist from that spray from going back upstream in the air flow.

The hot air with entrained water continues in a clockwise direction and passes through a mist eliminator **39**; which is in the form of a wire screening which removes the physical water droplets. It then re-enters the collecting and pre-mixing chamber **37** and becomes part of the intake air through the fan **41**. An exhaust duct **44** is provided with a damper valve **47** ostensibly to maintain positive pressure. It is stated that the pressure in the chamber **37** is above-atmospheric.

Intake air is supposedly controlled by the temperature of the exhaust gas in duct **43**.

The specification states that in its method form, the invention generally comprises the steps of placing charged batteries or plates in a drying chamber, providing a stream of substantially oxygen-free drying gas by mixing cold, substantially oxygen-free air at high humidity with hot, substantially oxygen-free combustion gases and passing the stream of drying gas through the drying chamber containing the battery plates to be dried. It states that the drying gases should be of a relatively low temperature to avoid injury to the charged battery plates; preferably not more than about 93°C (200° fahrenheit) or less; the preferred range being about 37.8°C to 121°C (100° fahrenheit to 250° fahrenheit) and preferably the temperature will be adjusted in the range of 77°C (170°F) to 85°C (185° fahrenheit). The specification states that the apparatus can be regulated accurately at 82°C (180° fahrenheit) if desired.

According to the present invention there is provided apparatus for drying charged battery plates having a housing capable of maintaining a positive gas pressure within it, a drying chamber within said housing having means for supporting battery plates to be dried in a position such that gas is allowed to move past the plates, a combustion chamber within said housing for providing hot, dry, substantially oxygen-free gas to a blower means for blowing the gas past said plates so as to effect drying of the plates by removing moisture therefrom, said apparatus characterized by:
water sheeting means for providing a flowing sheet of cooling water so as to contact the gas exiting from said plates and condense out the moisture removed from said plates during drying; and
temperature control means for maintaining a temperature differential within said drying chamber, said temperature control means minimizing the heat used to compensate for heat lost due to said condensation of moisture from the drying gas, so as to minimize the energy necessary to raise the temperature of the drying gas, thereby maximizing the thermal efficiency of said apparatus in drying the plates, said control means including air temperature measuring means upstream and downstream of the plates for controlling the temperature within said drying chamber.

Also provided according to the present invention is a method of drying charged battery plates comprising the steps of: placing the charged plates in an apparatus comprising a drying chamber, providing a flow of substantially oxygen-free drying gas of relatively low humidity directed to pass over said plates in order to effect drying thereof; condensing the water from the gas which has passed over the plates to dry them, said method characterized by the steps of:
passing that gas over the surface of a sheet of water flowing in a counter direction to the gas without introducing droplets of water into the gas; and
maintaining the temperature differential within said drying chamber such that heat is used primarily to dry the plates and minimally to reheat the air from the heat lost due to the condensation process in said method, by measuring the temperature of the drying gas before it is passed over said plates; measuring the temperature of the drying gas after it has passed over said plates; measuring the temperature of water exiting from said apparatus; and regulating the temperature and flow rate of said sheet of water in accordance with these measurements.

The essence of the present invention is that the energy input in the form of heat is controlled by both the apparatus and the process, to provide maximum thermal efficiency. Heat is used primarily to dry the plates and minimally to reheat the air from the heat (temperature) loss due to the condensation process. In the prior art, the apparatus and method, as exemplified by the Tiegel machine, used too much cooling, that is, more than what was needed. That machine used a spray nozzle, as well as very cold water. The spray nozzle caused high surface area water droplets which not only transferred heat quickly, but also created problems in that they were transferred to the plates, thereby lengthening the time it took to dry them. This created a need for even more kJ (BTU) to bring the machine up to temperature.

By the method, heat is used to remove the moisture from the plates and to bring the temperature from approximately 69°C (157°F) back up to 93°C (200°F). In the prior art Tiegel method, heat was used to remove the moisture from the plates and to bring the process air temperature to 82°C (180°F) from 49°C (120°F).

In this new method, the heat which is used for drying the plates reduces the temperature in the air from 93°C (200°F) to approximately 71°C (160°F). An additional 1.7°C (three degrees F) is used for cooling to remove the moisture from the air. Then it is brought back up to the process temperature of 93°C (200°F). This 1.7°C (three degrees F) is the only loss; that is, the only inefficiency. It is defined as a loss because it does not contribute to evaporating moisture from the plates. In accordance with the present invention, the apparatus and method uses 22°C (forty degrees F) of temperature change to do useful work, and 1.7°C (three degrees F) that does not do useful work. Thus the thermal efficiency is approximately 90%.

As a practical matter, the Tiegel machine went from 82°C (180°F) to 71°C (160°F) during the drying process, and then 71°C (160°F) to 49°C (120°F) during that portion of the process which cooled the air. Thus, the prior art machine had a 22°C (forty degree F) temperature drop; which was wasted energy. Its thermal efficiency was 11°C (twenty degrees F) for useful work and 22°C (forty degrees F) of wasted work for total energy consumption of 33°C (60 degrees F). Its thermal energy efficiency, therefore, was 11°C (twenty °F) divided by 33°C (sixty °F), or 33%.

Furthermore, because Tiegel kept re-introducing moisture into the plates, it took that machine an extended period of time to dry those plates. In actual tests, it appears that the time elapsed by the new machine is three times as fast as the time used by the Tiegel machine. Thus, on a comparative thermal efficiency basis, the prior art Tiegel machine has a comparative thermal efficiency of 11%. Some of the differences from the prior art dryer are as follows:
1. No spray nozzles, means not re-introducing water via droplets into the process.
2. No mist eliminators, means decreased back pressure.
3. No baffles, means decreased back pressure.
4. Higher thermal efficiency.
5. Plates which are dryer.
6. Lower oxygen levels in the plates.
7. Automatic drying to desirable moisture level in the plates.
8. No moving damper on the stack.
9. No freon temperature bulb.
10. An insert oven.
11. Improved flame rod.
12. Automatic pilot.
13. Automatic loading/explosion door.

The main advantages of the new dryer are:
1) reduced operating cost, which would be approximately the following:

| | OLD | NEW | ANNUAL SAVINGS (200 workdays/8 hr.day) |
|---|---|---|---|
| ELECTRICAL/HR | 28 KW | 3.0 KW | |
| | $4,480 | $ 480 | $ 4,000.00 |
| GAS: (BTU/HR) | (450,000) | (150,000) | |
| J/s | 131 882 | 43961 | |
| | $ 3,600 | $ 1,200 | $ 2,400.00 |
| COOLING WATER: | | | |
| (GALLONS/HR) | (900) | (420) | |
| l/hr | 3407 | 1590 | |
| | $1,440 | $672 | $ 728.00 |
| | | TOTAL SAVINGS | $ 7,128.00 |
| Notes: Electricity at 10 cents per KW hr. | | | |
| Gas at 50 cents per 105506 kJ (100,000 Btu) | | | |
| Water at $1.00 per 3785 l (1000 Gallons) | | | |

| Minutes to dry industrial plates: | |
|---|---|
| Old | 150. |
| New | 45. |

2) Higher reliability:
By measuring the temperature entering the plates and leaving the plates, dryness can be determined. A return temperature sensor determines if the cooling water is adequate in flow and/or low enough in temperature to remove sufficient moisture from the air before reheating. This allows just the right amount of cooling to be used throughout the drying process.
If a cooling tower is used, the fan is turned on only when increased flow does not produce enough cooling, and lower water temperature is required. Another method is to automatically blend the hot with the cold water coming from the cooling tower.

3) A safer machine:
The loading door is the explosion door which opens up, rather than to the side, as in the old style machines. In addition, the loading door is opened and shut with a pair of air cylinders (one located on each side). This prevents the door from flying open freely.

The flame monitoring is done under microprocessor control that opens the door when the flame rod detects a loss of flame. Therefore, the door is opened before an explosive condition can be created. Traditionally, when flame failure occurred, both combustion gas, and air were turned off immediately. This created an accident waiting to happen, because the combustible gasses were still in the oven. Therefore, the instant oxygen diffused into the firebox, an explosion or flash fire would occur. This would occur by just waiting long enough or by opening the explosion or loading door.
The Tiegel machine actually has a special solenoid to insure rapid air shut off. The new approach turns off the gas and flushes out the fire box with air before combustible gases have a chance to accumulate in the fire box. This is done by opening the combustion air to full open. At the same time, the loading door is opened to eliminate the containment necessary for an explosion.
4) Reduced maintenance by the elimination of many parts:
The new machine does not have the following parts:
   Mist eliminator screen: In areas with hard water, this screen would build up with calcium deposits that would have to be removed by soaking in hydrochloric acid annually. There was a pressure switch to indicate the mist eliminator was flooding due to deposits of water or calcium.
   Damper: This would stick over time. Also there was a sensor for this on the prior art machine. The new machine has no exhaust damper - only a short exhaust port that maintains positive back pressure, due to its restricted diameter.
   Spray Nozzles: There are no spray nozzles to clog, corrode, or wear out.
   Pressure Regulator: No pressure regulator is required to control flow. This is done with a motorized valve.
   Baffle plate: None is required because no water droplets are formed with the new cooling process.
   Fault finder to identity what failed: No fault finder is required because of the new flame control whereby, upon loss of gas or combustion air, a warning light comes on.
   Separate Explosion door: There is no separate explosion door or explosion door indicator switch. The loading door does double duty.
   Loading door latches: There are no loading door latches, because of reduced box pressure reduced from 380 mm (15 inches) down to a range of 31.75 mm to 63.5 mm (1.25 to 2.5 inches) water column. Pressure must be positive to prevent oxygen inflow. The air cylinders that open the door also act to hold the door shut during plate drying.
   Pilot button: No pilot button or manual gas valve, because the machine automatically establishes a pilot.

5) Other features:
My new insert oven comes in two parts: either one, or both, can be replaced in a matter of hours. The old machine required one to jack hammer out the old brick, re-brick, and allow the cement to cure. This process could take several days to weeks if the labor was not readily available.
The old machine used a mercury bulb to monitor temperature, which would leak from time to time. The new machine has a thermocouple probe.
The low wind velocity of the new blower is below 32 km/hr (20 mph), so the loading door can stay open during purge with the main blower running.
An automatic cooling control automatically turns on the cooling tower pump and/or fan to meet cooling needs.
A lower loading height that meets OSHA requirements for lifting baskets
Smaller components are needed to run the machine, e.g.:

| OLD | NEW |
|---|---|
| 22 kw (30 horsepower) main blower | 2.2 kw (3 horsepower) main blower |
| 22 kw (30 horsepower) motor starter | adjustable frequency AC drive |
| 100 amp circuit breaker | 10 amp circuit breaker |
| 745.7 W (1 horsepower)water pump | gravity feed |

6) Process improvements:
The new dryer achieves the same drying time with much less energy.

The Tiegel patent contains two false assumptions: first, that air can only be sufficiently cooled to remove moisture with the high surface area water droplets that the spray nozzles provide. In addition, it failed to recognize that if you cool the air beyond a certain point, you waste heat making hot water and do not hasten the drying process significantly . The spray nozzles created many problems whose solution created ever higher demands for electrical power. The same drying can be achieved merely by cooling with a thin film of water that flows from the rear of the machine to the front of the machine. It was also found that if the water flowed too quickly, the drying time lengthened rather than shortened.

Because no water droplets are formed, none can be blown about and reintroduced onto the plates. All the components needed to deal with the water drops created by the spray nozzles have been removed, such as the mist eliminator and baffle plate.

The back pressure dropped from 380 mm (15 inches) to 63.5 mm (2.5 inches).

A prototype machine incorporated a new high m³/s [cfm (cubic feet per minute)] low pressure design. The basket was redesigned to eliminate wind blockage while maintaining strength. This dropped the pressure even further, down to 31.75 mm (1.25 inches). The watts (horsepower) required to move a given m³/s (cfm)varies with the cube of the back pressure (static pressure). Thus, if the back pressure doubles, the watts (horsepower) needed for the same m³/s (cfm) increases four fold.

At the air flow being used, the air comes in to the plate at 93°C (200° F) and leaves at 71°C (160° F). If the exit temperature rises above 71°C (160° F), it means that the amount of moisture remaining is very little or there is insufficient cooling. There is just as much moisture in the air before and after going through the plates. If the temperature is much below 66°C (150° F), the air is very dry, but the drying is slowed, because most of the moisture is recondensing on the plates before leaving them.

The temperature of the air just before reentering the blower to be mixed with hot combustion air, should be about 67° to 69°C (153° to 157° F). This indicates that moisture removal from the air is adequate.

If the exit water temperature of the cooling water is 60°C (140° F), significant increases in drying time are noticed. If the temperature is at or about 46°C (115° F), the cooling is just enough. Otherwise, it is just a waste of cooling capacity and heat. Therefore, by measuring the cooling water temperature entering and leaving the machine and its flow rate the amount of heat leaving the dryer via the water can be determined. Per experiments, the temperature entering is 29°C (85° F) and leaving is 46°C (115°F), with a flow rate of water which is modulated to keep the water leaving at 46°C (115°F); on the average this is 0.76 ℓ/s (10 gallons per minute). This translates into a heat transfer of about 41030 J/s (140,000 Btu per hour) to the water.

### DISCLOSURE OF THE INVENTION

### BRIEF DESCRIPTION OF DRAWINGS

Figure 1 is a drawing from prior art patent 3,413,728 showing a vertical section taken through the machine described in said patent, substantially in the plane taken as indicated by the lines and arrows 1-1 in Figure 2;
Figure 2 is a top section view of the machine shown in Figure 1 with the cover removed in order to illustrate internal parts; the view being indicated as taken by the lines and arrows 2-2 in Figure 1;
Figure 3 is an enlarged cross-sectional view illustrating in greater detail the placement of charged battery plates in the apparatus as shown in the prior Figures;
Figure 4 is a vertical section of a machine in accordance with the present invention taken as in Figure 1;
Figure 5 is a top view, partially is section, taken as a view similar to that shown in Figure 2 of the prior art;
Figure 6 is a view similar to Figure 4, except it is taken from the opposite side and is an external elevation;
Figure 7 is a front elevation taken as indicated by the lines and arrows 7-7 in Figure 5.
Figure 8 is an exploded perspective view of a portion of the apparatus comprising the firebox shown in Figure 5;
Figure 9 is an enlarged view of a portion of the apparatus comprising the flame rod shown in Figure 5;
Figure 10 is a psychometric chart; and
Figure 11 is an enlarged view of a portion of the apparatus comprising an oxygen sensor.

### DESCRIPTION OF THE PREFERRED EMBODIMENTS

Referring to the Figures, the invention comprises structural elements which are shown in Figures 4 through 9, namely there is a housing **10** made of stainless steel (shown in Figure 4 with the side wall removed), which has a door **12** which provides a closure for an opening through which the baskets **14** containing the groups of charged battery plates to be dried may be lowered into the chamber **16** for drying. At the rear of the chamber **16** there is a blower, designated generally **17**, for forcing hot air from the rear down into the chamber **16** in the direction of the arrow **A** shown. There is a heater, designated generally **21.** Below the baskets, there is another chamber **22** which has an upper bed **24,** preferably being of stainless steel, which extends from side to side within the chamber **22**, but does not extend from the front to the back of the housing **10**. Water is introduced at the bed's upper end **23** through inlet piping, **26**.

There is also a lower bed **29** positioned below the upper bed and extending forward of the upper bed as illustrated in Figure 4. The lower bed also has water introduced by means of piping **30** at its upper end designated generally **32**. Positioned running the length of each of the beds are a plurality of angled strips **34**, **36** having their longitudinal bottom portions welded to the stainless steel beds **24** and **29** respectively, so that there is formed a plurality of flat channels designated generally **35** therebetween as clearly illustrated in Figure 5.

Across the bottom edge of each of the beds is another angle shaped member **31, 40** respectively positioned and dimensioned as shown in Figures 4 and 5.

The pipes **26** and **30** run along the entire width of the beds **24** and **29** respectively, and have a plurality of holes for introducing the water. In order to cut down on the splashing of the water, the holes communicate with flat webs **42, 43** respectively, so that the water introduced through the pipes runs down the flat webs and onto the upper surfaces of the beds without splashing.

In operation, when the air progresses from the chamber **16** to the chamber **22**, it would normally tend to blow the water up the sloped beds **24, 29** and indeed the slopes are arranged at an angle such that the water will eventually build up on the beds so that the static head will overcome the force of the air blowing the water up. Most preferably, the water is introduced and the air is moved at a rate such that the contact between the air and the water is just below that which would cause "white caps". The desire is to keep water particles from being entrained in the air. The angle members are positioned and arranged, as are the beds themselves, so that water collects along the members **31** and **40** Figure 4 and exits at the edge closest to the walls **46** and **48** as, for example, in the spaces or slots designated generally **50**, **52, 54** and **56** in Figure 5. The flow of water and the spaces are dimensioned and designed such that the water simply runs down the sides, rather than dropping as a waterfall. A waterfall would cause undesirable splashing and water entrainment in the air. The water is collected in a trough, **58,** Figure 4, from which it leaves by means of gravity into a sump (not shown) and is pumped back to a cooling tower to be thereafter reintroduced into the machinery.

It will be appreciated that the two beds of flowing water create a much greater surface area for heat transfer than the flat beds themselves, due to the counter flow temperature gradient.

The entire chamber is insulated, which makes it possible to operate at a higher temperature and, therefore, reduce drying time of the prior art devices.

The long fins, or angled members **34, 36**, keep the water controlled, that is, keep it from scooting out of the way when the blower is on, and thus keep a wetted surface on the beds.

Slots designated generally **51** on the bottom of the angled members allow the water to exit from each channel.

Turning now to the heating and blower arrangement, the heating chamber **78** is insulated on all sides, Figure 5, with the exception of several ports. An internal wall **60** in the fire box, Figure 5, contains the heated air and channels it to approximately the center of the fire box heating chamber **78**, where a portion of it continues to move forward and out the port, designated generally **61** in Figure 5. The remainder is channelled around the wall **60** and exits through the port, designated generally **64.** The heated air passes into the chamber **66** Figure 7 from whence it is sucked into the suction ports designated generally **68** and **70** of the twin rotor blower designated generally **17**.

The blower blows the air out through the orifice, designated generally **72.** The panels **74** and **76** engage the side walls and top of the housing forming chamber **16,** to form an expanding chamber for introducing air on top of the plates.

While there is now a greater m³/s (cubic feet per minute) possible, the air tends to stay in the closed loop in the machine. In the prior art, the baffle plate tended to divert the air out of the machine. Therefore the top front door had to be closed during preparation prior to introduction of the combustible gasses. Accordingly, purging was necessary because of gas leaks and human error. When the machine was idle in the prior art, the purge time was two minutes. The purge time in the present machine is approximately twenty seconds. In this machine, all one does is turn it on and flush it with four volumes of air for that preset time. The machine is set to go to a lower speed, so that there can be combustion when the operator hits the start button to start the process. Once the door closes, the main blower comes on and the drying process starts.

The machine measures the temperature below the plates by the thermocouple **88,** Figure 4. Once that gets to 57°C (135° F) (below that there is insufficient evaporation from the plates) water begins to flow in at approximately 24°C (75° F).

The temperature going into the plates is measured by the thermocouple **86**, Figure 4. When these temperatures are close, the plates are dry. Normally, there is a 5.6°C (10° F) differential at the point at which the plates are just about dry. This can be adjusted. This prevents thermal "run away", wherein the machine thinks the plates are dry and shuts down.

By means of the thermocouple **90**, the water temperature leaving is measured at 46 to 49°C (115° to 120°F). This reading is used to modulate the water and, therefore, the cooling flow.

The process of evaporation extracts 19 to 22°C (35° to 40° F) of heat. Water leaving the plate, gets condensed into cooling water as previously stated, and goes to the cooling tower.

When the plates are dry, the machine shuts down to a "ready to process" phase, in which condition there,is a pilot light still lit. The door then opens automatically.

A number of items of improvement over the prior art are in the most preferred embodiments. For example, a quartz tube **110** is put over the flame rod **108** to keep it hot, that is above 100°C (212° F), and thereby prevent condensation which would inhibit electrical grounding. See Figure 9.

The exhaust gas outlet stack **89** Figure 4 is placed near the rear of the machine proximate to the drive shaft of the blower, that is, at the lowest pressure point. Thus, the exhaust gas at this point is close to "zero" pressure, whereas the pressure at the outer periphery of the blower is 38 mm (1.5 inches) of water. Note in this regard that if the exhaust stack was placed at the top, there would be minus 38 mm (1.5 inches) at the shaft and air could be sucked in. In the prior art, the exhaust stack was just after the spray nozzles on the side, and on the suction side of the main blower, before the mist eliminator. Any place in the prior art machine that there was a blockage, there was also a pressure drop. This created an even more negative pressure within the prior art machine and, therefore, the stack required a damper with a counter weight on the top (see 47, Figure 1 of the prior art) to make sure the pressure did not go negative. Also the machine required a sensor to shut it off.

Herein, the pressure is read right at the fire box and thus, the machine senses if the box is going to negative pressure. If so, the machine automatically shuts off the fire.

A zero governor is connected to the manometer to mix the gas and air.

Since the rear explosion door of the prior art machine has been eliminated, this also eliminates the prior art rear door seal, which was a problem insofar as there was air leakage around the door. This would mean that additional oxygen would get in and cause damage to the product being processed.

The machine is designed to run the burner at 100% perfect ratio, so that all the oxygen is burned. This is possible so long as air is not sucked in from the outside. Thus, it is necessary to maintain the pressure so that the machine does not go to negative pressure.

To aid in this, an air seal is provided around the top front door, which is maintained in tight communication with adjoining upper walls by air cylinders on the sides of the door. These air cylinders keep pulling down against the door in order to maintain the seal.

The controls are set up such that the instant the flame rod says there is no flame, the front door opens.

In the prior art, the water discharge was 152 mm (6 inches) from the input. In the present machine, it goes the length of the machine away from the output.

Some salient features of this dryer are as follows:
1/6th of the energy used by the blower as compared to the prior art.
No spray nozzles for cooling of the water and no mist eliminator. The hot moist air comes in direct contact with the water film on the beds which cools and condenses it, and the condensed moisture is entrapped into this film.
Because of the limited surface area of the water film, the hot gasses leaving the plates are not excessively cooled and thereby reducing the load on both the cooling water and the burner.
The water is not turned on until a given temperature has been reached; for example, 57°C (135°F). The flow can be modulated down to almost no flow of water at the end of the cycle (when there is very little moisture to remove) and the exit water temperature most preferably never goes below 46°C (115°F).
In the morning the machine is turned on. The door is already open. The process blower for the furnace comes to top speed with the butterfly valve in the air input of the burner open, to automatically purge the machine of combustible gases in approximately 20 seconds. Then the butterfly valve closes to the low fire position, the main process blower turns off, and then the pilot gas and ignition transformer turn on simultaneously for about 15 seconds. If ignition is successful, plates can be loaded. When it is turned on, the main flame is growing. Approximately five seconds later, the operator can then press the start button which will automatically close the loading door. After about ten seconds the main burner comes full on. The process then continues until the temperature reaches above 81°C (180°F) whereupon the water is turned on. This permits a rapid heating up of the product without the unnecessary cooling of the drying gases. At that point, the water is being drawn out of the drying environment and this continues until the effective wet bulb temperature starts to rise up to approximately 77°C (170°F). From there the temperature rises quickly which indicates that the product has no moisture left to cause cooling of the process air. When the process air below the plates reaches 80°C (176°F) the plates are considered dry; although in practice the spread can vary. The process then automatically stops, and the loading door opens up to permit the operator to remove the product.
The drying process is controlled by the differential between the drying temperature and the wet bulb temperature. As long as the hot moist air contains moisture there is an excellent heat transfer between the water film and the drying gases. Once the water has been removed from the product, the air becomes dry and the actual heat transfer becomes quite limited on the water film.
The stack has been moved from the wet section to an area close to the entrance of the blower; which is the low pressure portion of the machine. The orifice is so positioned as to reduce the amount of hot air going up the stack. In actuality, the temperature of the exhaust gases is slightly less than the gas below the drying elements. The stack 89 contains a fixed reduced orifice thereby producing a positive pressure in the chamber.

Insofar as the energy conversion is concerned, note the following comments:
The rate of heat input to the plates is governed by the temperature and flow rate of air across the plates. Heat capacity of air or water vapor is about 0.5365 kJ/m³ (.0144 Btu per cubic foot) per 0.56°C (1° F)temperature change. For example, to raise 0.03 m³ (one cubic foot) of air 5.6°C (10°F) requires 0.152 kJ (0.144 Btu) of energy.
However, to convert liquid water to 0.03 m³ (one cubic foot) of water vapor requires 39 kJ (37 Btu). This is 256 times more energy. Therefore, the process of changing water to vapor or liquid to vapor dominates the heat transfer process. A small decrease in the temperature of 100% water vapor saturated air translates into a large transfer of energy. For example, changing the temperature from 68.3° to 65.5°C (155° to 150° F) in 0.03 m³ (one cubic foot) of water vapor saturated air releases 49.9 kJ/m² (1.34 Btu per cubic foot) of air. To get the transfer of the same amount of kJ (Btu) to air which is not 100% water vapor saturated, you would need a temperature change of 52°C (93°F) per 0.03m³ (cubic foot) of air. Bearing this is mind, it is theorized that there is a large temperature difference above and below the plate where the heat content of the air is used to evaporate the water from the plates. Whereas the temperature change of the air to condense the water vapor leaving the plates is much smaller because a much smaller change in 100% relative humidity (RH) air releases the large energy of condensation.
The energy profile of the dryer may be understood by reference to conditions in the chambers. Below the blower 68.3°C (155°F), 100% RH air is mixed with hot combustible air exiting from the fire box. The resulting air becomes 93°C (200°F) 35% RH air leaving the blower and moving into the chamber 16. In the chamber 22 right under the basket there is 71°C (160°F) at a higher RH (relative humidity). As the air travels above the water, to the rear of the chamber **22** there is a drop to 68°C (155°F) 100% RH air.
   Notice that the first process of the plate evaporation requires a 14° to 19°C (25°F to 35°F) change and the second process of condensation requires only a 1° to 4°C (2° to 7°F) change; even through the same amount of energy is being transferred. The total energy transferred via the air is proportional to the temperature change of the air. The total reheat requirement is equal to the sum of the ranges.
The last consideration is the m³/s (cubic feet per minute) of the main blower air. This is limited to the speed at which white caps are formed, since with the creation of white caps comes water droplets which are reintroduced into the plates.

A wind velocity meter measures the speed of the air past the cooling beds and changes the speed of the impeller so that the air speed remains constant. This means one can always dry as fast as possible. If there is a light load in the machine, the blower runs slower. If the plates are packed, it runs faster.

When the difference between the temperature of the air entering the plates and the temperature of the air leaving the plates goes below a certain point, the plates are declared dry. By keeping the exit water temperature constant at 46°C (115°F) (a temperature which was determined experimentally), the automatic dry temperature differential mentioned above can be detected. This is greatly different from the prior art in which, if the cooling water is too cold, the temperature never gets to the autodry differential. If on the other hand, one would back off on the water to too great a degree, the temperature reading would tell one that the plates were dry, when in fact they weren't. It is theorized that this is because one is measuring a very small level of moisture in a very active environment.

The prior art Tiegel machine had no insulation surrounding the fire box. This lead to uneven heating of the plates, because the plates near the fire box were heated both with a radiant heat from the fire box and with hot air. Thus, the plates near the fire box got too hot and the plates far away were too cold for maximum drying speed. Consequently, Tiegel recommended 82°C (180°F) as the most preferable operating temperature, while it is now possible to recommend a drying temperature of 93°C (200°F) as a result of insulating the fire box. This allows a process temperature twenty degrees higher than with the Tiegel dryer and thus allows a faster drying of the plates with no decomposition or auto-ignition problems.

An exploded view of the firebox construction is shown in Figure 8. Therein it will be noted that the box has been made in separate parts which are assembled and insulated, and then slid into a stainless steel sleeve **100.** The parts of the firebox comprise the input section **102,** the gasket **104** and a terminal section **106,** all made of a pre-cast, heat-tolerant material. The sections are assembled together and wrapped in insulation (not shown), then slid into the sleeve as shown in the assembled condition in Figure 5. Therein, the insulation is designated 62.

At the input section, there is a flame rod, **108**, Figure 9. A portion of the flame rod is covered with an extended hollow quartz tube **110**. It is theorized that the way the flame rod works is that one impresses a 250 AC voltage on it. The gas within the flame coming out of it is considered ground. As a flame is being lit, it ionizes the gasses and, because the wire is so, small in surface area compared to the ground surface, it becomes a semi-rectifying circuit. It is this half-wave rectification that is being monitored. If it becomes an AC (alternating current) wave, the monitoring circuit automatically rejects it and shuts the gas line down. In the previous art, what normally happened was that the porcelain insulation at the upper end would become wetted with moisture, and this would then form a circuit between ground and the high voltage. The AC would not be rectified, and, therefore, shut the gas line down. By means of this quartz tube, I have lengthened the leakage path.

At the other end of the firebox, there is a hole designated generally **111** through which is mounted an oxygen sensor **112**, shown in enlarged view in Figure 11. Such a sensor is very sensitive to both oxygen and carbon monoxide. Once there is a carbon monoxide present in the atmosphere, the voltage reading rises quickly. With a 60 millivolt reading, one can obtain zero percent oxygen.

A similar oxygen sensor **114** is also provided in the stack **89**, Figure 4 in the end of the tube **115** which is open proximate to the axis of the blower. The sampling tube **115** communicates through the bottom of the stack and is opened all the way up to the sensor **114** for purposes of measuring oxygen content. This provides the worst possible reading, since it is located proximate to the axis of the blowers **17** and, therefore, would be sensing the most negative pressure.

Another sensor **116** is mounted in a hole in the top of the stack 89 for the purpose of sensing temperature in the exhaust gas in case of a thermal runaway. At this point it will sense hot exhaust gas and shut the machine down.

The positioning and design of the stack **89** has been changed from that shown in the prior art, as will be appreciated from viewing the position of the stack **44** in Figure 1 and that of the stack **89** in Figure 4. The stack has been moved away from the blower/heat entrance. Furthermore, a restricted opening, designated generally **118** is provided also oriented away from the heat entrance from the firebox **78.** The restricted opening **118** is positioned so that it does not entrain the hot gasses coming from the burner. This restricted opening, and positioning prevents the monitor **116** from picking up an erroneous reading of a thermal runaway.

The use of these sensors is for monitoring the process. The sensors **112** and **114** are standard parts used in automotive gas exhaust monitoring systems.

One step in the process is to remove the water vapor from the air as the water vapor saturated air leaves the plates. The water vapor removal rate must be as fast as the water vapor leaves the plates. If it is too slow, the drying process slows and eventually stops, since the air becomes saturated with water. The new machine takes an entirely different approach in this step. Only a small temperature drop is required to remove an inadequate amount of water vapor via condensation. Any further cooling of air is a fruitless exercise. Thus the new dryer uses just enough cooling to maintain evaporative equilibrium. It has been found that a falling film of water introduced at 26 to 29°C (80° to 85°F) and leaving at 43° to 46°C (110° to 115°F) was quite adequate. The only requirement was that all the air needed to be cooled by similar amounts. Otherwise, the hot air would not cool and condense out the moisture; thus producing a mixed result. Therefore, most preferably the machine should contain a second falling film in the middle to further improve the drying speed.

Flow is modulated to keep the water exit temperature from the dryer at 46°C (115°F). In order to refine this process, cooling is not started until the temperature of the air leaving the plates is above 57°C (135°F). Below that temperature, the plates are not hot enough to release significant amounts of moisture. Cooling at the start of the drying cycle only increases drying time because it takes longer to come up to process temperature. Modulated flow of cooling also decreases the time to come up to process temperature and allows a more accurate determination of dryness. Therefore, plates are dried just enough. Historically, plates were always overdried just to make sure. Plates that were too wet, had to be formed, washed and dried all over again.

In the prior art, removing the last bit of moisture took over half the dry cycle time. This occurred because water droplets from the cooling spray nozzles were constantly being reintroduced into the plates being dried. The new dryer never creates water drops to start with. The falling water film clings to the cooling pan. The only way to create water drops in the new dryer is to move the air fast enough to create "white caps". Therefore, increasing m³/s (cubic feet per minute) can actually increase drying time, by creating "white caps". Thus, the air speed is set so that no "white caps" are formed.

The new dryer produces a product that has half the moisture content, in one third the time. This is achieved, in part, by not creating water droplets in the dryer that can be blown around and reintroduced into the product being dried. Further, it has been observed that the lead oxide content is also cut in half. This leads to a superior quality negative plate. The lower lead oxide level stems from faster drying, a tighter no leak oven and "on" air/gas ratio burning at a low firing rate. The new dryer also achieves this by using approximate atmospheric pressure as the reference for the zero governor. Since this approximate atmospheric pressure changes very little, the zero governor can continue to accurately dispense gas with a pressure differential of less than 12 mm (half an inch)water column. Ideally, one would want the gas pressure at the burner mixer to be equal to the pressure in the combustion chamber. The control, or governor in the gas input line, monitors this and controls it. The old dryer needed a pressure differential of more than 3 inches water column. If the damper got stuck in the closed position, the machine would pump in too much gas, creating explosive conditions.

Since the loading door is the explosion door as well, and the blower shaft is mounted on the flange style outboard bearing, the two major sources of oxygen intrusion have been eliminated. The oxygen usually would get sucked in via the main blower shaft where the pressure is the lowest and the seals are sloppy. The new dryer has the exhaust port right at the main impeller shaft. This eliminates the need for a damper and allows the fire box to run near atmospheric pressure. This also gives a very accurate "on" ratio burning, especially at low firing rates.

The machine is more user-friendly for the following reasons:
1. Auto Pilot. When an operator turns on the machine, the dryer automatically purges the whole oven of any combustible gases in less than 30 seconds by having the loading door open, the main blower 16990 m³/s (10,000 CFM) on and the combustion butterfly valve open. After the purge cycle is complete it automatically turns off the main blower and drives the butterfly valve to low fire. Once this happens the pilot is ignited automatically. The moisture proof. flame rod assembly prevents false lack of flame signal due to moisture. If ignition is successful a green ready light comes on. The dryer is ready to process plates with the turn of just one switch.
2. Auto Process - To process plates the operator loads them into the dryer and hits the process starter button. Then as the loading door automatically closes, the burner comes up to high fire. When the loading door is completely closed the main blower automatically comes on line. A white light comes on letting the operator know the plates are dry and that the loading door will open in less than 30 seconds indicating the plates are ready to unload. There is no process clock to set, because the dryer always knows when the plates are just dry enough. The operator can dry plates with the press of a button. There is no main gas valve handle to move or explosion door to close or loading door to latch.
3. Autodry/Auto Cool - These features work together to dry the plates as fast as possible to the same level of dryness every time. They keep cooling and gas consumption to a bare minimum. "Auto dry" determines the exact point of when the plates are dry and "auto cool" introduces just enough cooling to remove moisture as it leaves the plates. Cooling is reduced as the amount of moisture leaving the plates declines. Auto dry automatically compensates for poor basket packing by increasing the dry time. It also adjusts for changes in product type. The operator can choose the level of dryness he wants by changing the "autodry" set point. Maximum production speed is achieved all the time. There is no guessing at proper drying time.
4. Automatic adjustment of blower speed to compensate for back pressure differences when one changes from group drying to cassettes or rack drying. The wind speed is always just below white cap formation speed. This further maximizes drying speed of what is being dried.
5. The control box displays process air, exhaust stake, "auto dry" and water outlet temperature which allows the operator to detect and correct malfunctions, such as lack of cooling, without the machine shutting down while processing plates. This eliminates unnecessary product loss. Cooling tower status is also indicated.
6. A white light turns on, warning the operator that the loading door will be opening in less than 20, seconds.
7. Quiet machine. Only 3dB (decibel) over factory background noise.
8. Low profile machine. Bottom basket level to clear loading entrance is less than 50" from ground level.

### MORE UTILITY EFFICIENT

1. Electric: 3.0KW
2. Gas: 73268 J/s (250,000 Btu/hr)
3. Water: 1590 l/hr (420 Gallons/hr).

When one factors in the three-fold increase in drying speed, the utilities become the equivalent of 1.0KV, 24325 J/s (83,000 Btu/hr) and 530 ℓ/hr (140 gallons/hr).

### MORE MAINTENANCE FRIENDLY MACHINE

1. No mist eliminator screen to clean.
2. No spray nozzles to wear out or clog.
3. No exhaust port damper to stick.
4. Main blower bearing mounted externally.
5. No re-bricking. Insert firebox modules.
6. No explosion door seals to maintain.
7. No fault finder box.
8. No freon bulb to calibrate or replace.
9. No paint. All fixed parts 316 stainless steel.
10. No basket baffle plate.
11. No basket seal to maintain.
12. No explosion doors to maintain.
13. No zero governor feedback tube to clog zero governor with moisture and firebox material.
14. No fan belts.

It is further theorized that this machine is much more efficient because, as one can see from the accompanying psychometric chart, Figure 10, by going to the higher temperatures, namely 82°C (180°F), the amount of humidity that can be put into the pound of dry air goes up quite rapidly. It is virtually a logarithmic function, which flattens out as one comes down to approximately 54° to 49°C (130° to 120°F). Cooling below this point serves a very limited purpose. The change from a vapor state to a liquid state happens at the same temperature and, therefore, a 1.7°C (3°F) change is able to transmit alot of energy into the water.

In summary, one wants to have the air hot enough in temperature in order to load it up with sufficient moisture and cool it just sufficiently enough to condense the moisture out without unnecessary cooling. As one can see, the drop of temperature from 78.3 to 76.7°C (173° to 170°F) would change the humidity from 0.218 kg (.48 lbs) of water per 0.45 kg (lb) of dry air, down to less than 0.195 kg (.43 lbs) This compares to a 2.5 fold difference if one were at 54°C (130°F) temperature where there would be approximately 0.064 kg (.14 lbs) of water per 0.45 kg (pound) of dry air falling down to only 0.054 kg (.12 lbs) of water per 0,45kg (pound) of dry air at 54°C (130°F) temperature. Thus, the process and machinery work up in the 78°C (173°F) region in order to increase the efficiency. From this it can be seen that in the prior art they had to decrease the air temperature to keep the plates from decomposing as they would at a temperature over 104°C (220°F). Now we can uniformly dry at essentially 92.2° to 93.3°C (198° to 200°F.)

The maximum use and efficiency of this apparatus has been further increased by redesigning the baskets and the method and means by which they are inserted and withdrawn. Figures 4 and 5 show the basket in elevated and plan views. Each basket **14** consists of an open frame which has an internal ledge **120** upon which are placed a series of tubular structures **122** which are essentially rectangular in cross-section. On the upper surfaces **124** there is a plastic strip having transverse serrations. The serrations are used to space battery plates longitudinally. The tubular structures **122** are movable along the basket ledge **120** in order to accommodate various widths of battery plates. It is understood by those skilled in the art that battery plates have tabs extending from them and that these tabs can be placed within the individual serrations in order to space the plates. Each end of the basket has a stainless steel inverted "V" shaped wire member **126** round in cross-section welded thereto; so that the upstanding apex of the "V" is located substantially on the center line of the basket. In order to withdraw the baskets, a rod **128** which has two hooked-shaped members **130, 132** welded to it is inserted down between the outermost edge of the basket and the inside sidewall of the housing **10**. This rod is then rotated 90° and lifted upwardly so that the hooks engage the respective apexes of the "V" shaped handles of the baskets **14.** The hooks are placed a greater distance apart than the upstanding "V" shaped apexes so that the top hook engages first and begins to lift the top basket before the bottom hook engages and lifts the bottom basket. This basket design not only aids in air flow, but also in maximizing the number of plates that can be placed in a standard sized vessel. Furthermore, the basket is so dimensioned that there is only a slight clearance for the rods **128** to come down and engage the hooked-shaped members. This also aids in removing the baskets in that they will not, in practice, cock and jam upon withdrawal.

## Claims

1. Apparatus for drying charged battery plates having a housing (10) capable of maintaining a positive gas pressure within it, a drying chamber (16) within said housing having means (14) for supporting battery plates to be dried in a position such that gas is allowed to move past the plates, a combustion chamber (21) within said housing for providing hot, dry, substantially oxygen-free gas to a blower means (17) for blowing the gas past said plates so as to effect drying of the plates by removing moisture therefrom, said apparatus **characterized by**:
water sheeting means (24, 26, 29, 30, 34, 36) for providing a flowing sheet of cooling water so as to contact the gas exiting from said plates and condense out the moisture removed from said plates during drying; and
temperature control means for maintaining a temperature differential within said drying chamber, said temperature control means minimizing the heat used to compensate for heat lost due to said condensation of moisture from the drying gas, so as to minimize the energy necessary to raise the temperature of the drying gas, thereby maximizing the thermal efficiency of said apparatus in drying the plates, said control means including air temperature measuring means upstream (86) and downstream (88) of the plates for controlling the temperature within said drying chamber.

2. The apparatus of Claim 1, wherein the combustion chamber comprises a firebox (78) in the combustion chamber (21), said firebox (78) including a casing (100) having removable inserts (102, 106).

3. The apparatus of Claim 2, wherein the removable inserts (102, 106) are configured to provide communicating chambers, said chambers channeling the hot, dry air to two exhaust ports (61, 64) proximate to the walls of said housing (10), said exhaust ports being spaced from one another.

4. The apparatus of Claim 2, wherein the removable inserts (102, 106) also comprise a spacer (104), said spacer (104) and said inserts (102, 106) being insulated (62) from the firebox casing (100).

5. The apparatus of Claim 2, wherein the firebox (78) has a flame rod (108) with a quartz tube (110) extending around said flame rod (108) over the greater portion of the length thereof.

6. The apparatus of Claim 2, wherein an oxygen sensor (112) communicates with said firebox (78).

7. The apparatus of Claim 1, wherein the water sheeting means provides a sheet of water flowing in a counter direction to the flow of air and includes at least one bed (24, 29) positioned below said plates in said housing (10) on an angle to provide gravity feed of said water; said bed having fins (34, 36) thereon directing the water into separate webs (35) thereof.

8. The apparatus of Claim 7, wherein water is introduced along an upper portion of said bed by a header pipe (26, 30) having a plurality of holes therein communicating with a vertically upstanding web (42, 43) such that the water runs smoothly onto said bed without splashing.

9. The apparatus of Claim 7, wherein said bed terminates in a retaining wall (31, 40) and slots (51) are provided in said fins (34, 36) to allow water to exit off of said bed and said webs (35).

10. The apparatus of Claim 7, wherein said water drains into a trough (58) and a temperature sensor (90) is positioned in said trough to measure the temperature of the water exiting from said trough (58).

11. The apparatus of Claim 1, wherein said blower means (17) comprises blowers mounted on a shaft, said shaft being supported by bearings (79) mounted externally on the housing.

12. The apparatus of Claim 1, wherein said blower means (17) comprises at least one blower mounted on an axis positioned downstream of the hot gas exiting the combustion chamber, and a stack (89) is provided positioned posterior to the axis of the blower, said stack (89) having a restricted opening (118) at its lower end positioned to open to the rear of the housing away from the hot gas exiting from the combustion chamber.

13. The apparatus of Claim 12, wherein a temperature sensor (116) is provided at the top of said stack (89) external to said housing (10).

14. The apparatus of Claim 12, wherein a hollow tube (115) is positioned within said stack (89) having one end communicating with said apparatus at approximately the plane of the axis (79) of the blower means (17) and the other end communicating through the external end of said stack (89), and an oxygen sensor (114) is mounted in said one end of the hollow tube (115) opposite from the end external to said housing (10).

15. The apparatus of Claim 1, wherein the means to support the battery plates to be dried comprises at least a basket (14) having a ledge (120) upon which adjustably movable racks (122) are positioned so as to retain said plates.

16. The apparatus of Claim 15, wherein said racks (122) have serrated upper surfaces (124).

17. The apparatus of Claim 15, wherein said baskets (14) have handles (126) thereon comprising inverted "V" shaped rods affixed thereto; and removal means (128, 130, 132) are provided to engage said "V" shaped handles for lowering said basket into said housing or removing said basket from said housing.

18. The apparatus of Claim 17, wherein said removal means for lowering or removing the basket comprises a rod (128) having at least one hook (130, 132) thereon, said rod being positioned and dimensioned so as to fit between the inner wall of said housing and the outer wall of said basket, so that after the rod is inserted therein and then rotated, upon removal said removal means engages said "V" shaped portion of said handle (126).

19. The apparatus of claim 18, wherein a plurality of baskets are used in said apparatus and the hooks (103, 132) on said removal means are spaced apart from one another a greater vertical distance than the vertical spacing of the "V" shaped handles (126) when said baskets are stacked upon one another, so that when said rods (128) are rotated and withdrawn, an upper hook (130) engages the upper "V" shaped portion of an upper basket handle before the lower hook (132) engages the "V" shaped portion of the lower basket handle.

20. The apparatus of claim 1, wherein said apparatus is provided with a door means for opening into said housing so as to permit baskets to be lowered into said chamber, and for closing to permit said apparatus to function in the drying process, said door means having a door being hinged along one edge thereof and having one or more piston and cylinder arrangements attached to said door and to said housing to actuate said door.

21. The apparatus of claim 20, wherein said door means has a door (12) with a seal around the edge thereof mating with said housing to prevent oxygen leaking in during the processing function of said apparatus.

22. A method of drying charged battery plates comprising the steps of:
placing the charged plates in an apparatus comprising a drying chamber (16), providing a flow of substantially oxygen-free drying gas of relatively low humidity directed to pass over said plates in order to effect drying thereof; condensing the water from the gas which has passed over the plates to dry them, said method **characterized by** the steps of:
passing that gas over the surface of a sheet of water flowing in a counter direction to the gas without introducing droplets of water into the gas; and
maintaining the temperature differential within said drying chamber such that heat is used primarily to dry the plates and minimally to reheat the air from the heat lost due to the condensation process in said method, by measuring (86) the temperature of the drying gas before it is passed over said plates; measuring (88) the temperature of the drying gas after it has passed over said plates; measuring (90) the temperature of water exiting from said apparatus; and regulating the temperature and flow rate of said sheet of water in accordance with these measurements.

23. The method of claim 22, wherein the temperature of the water exiting is maintained in the range of 46° to 49°C (115° to 120°F) and most preferably at 46°C (115°F).

24. The method of claim 23, wherein the gas flow over the surface of the sheet of water is regulated so that it is below the rate which would cause "whitecaps".

25. The method of claim 22, wherein thermal runaway is prevented in said machine by sensing (116) the temperature of the hot gas in the blower chamber by passing that gas through a restricted opening (118) proximate to the axis of blowers (17) in the machinery and reading the temperature externally of the apparatus.

26. The method of claim 22, wherein said drying gas is heated in a confined area and the oxygen content in said gas is measured at said confined area and exiting said confined area.

27. The method of claim 22, wherein the method of heating and drying plates comprises confining the plates in a closed area (10) which has first been purged of combustible gases and heating the air in said closed area until the temperature reaches above 82°C (180°F), and then introducing said sheet of water.

28. The apparatus of claim 1, wherein the sheet of water flows in a counter direction to the gas exiting from said plates.

29. The apparatus of claim 1, wherein there is provided a plurality of sheets of water for contacting said gas exiting from said plates.

## Patentansprüche

1. Vorrichtung zum Trocknen geladener Akkumulatorplatten, die ein Gehäuse (10) hat, worin ein Gasüberdruck aufrecht erhalten werden kann; mit einer Trocknungskammer (16) im Inneren des Gehäuses mit einer Vorrichtung (14), um die zu trocknenden Akkumulatorplatten in einer solchen Position zu halten, dass Gas hinter die Platten strömen kann; mit einer Verbrennungskammer (21) im Inneren des Gehäuses zum Bereitstellen von heißem, trockenen und weitgehend sauerstofffreien Gas für eine Gebläsevorrichtung (17), um das Gas hinter die Platten zu blasen, um ein Trocknen der Platten durch Entfernung von Feuchtigkeit davon zu bewirken; welche Vorrichtung **gekennzeichnet ist durch**:
Wasserschleier-Vorrichtungen (24, 26, 29, 30, 34, 36) zur Schaffung eines strömenden Schleiers von Kühlwasser, um so mit dem aus den Platten austretenden Gas in Kontakt zu gelangen und die von den Platten während des Trocknens entfernte Feuchtigkeit zu kondensieren; und
Vorrichtung zur Temperaturregelung für die Aufrechterhaltung einer Temperaturdifferenz innerhalb der Trocknungskammer, wobei die Vorrichtung zur Temperaturregelung die zum Ausgleich des Wärmeverlustes infolge der Kondensation von Feuchtigkeit aus dem trocknenden Gas aufgewendete Wärme auf ein Minimum herabsetzt und damit die zur Erhöhung der Temperatur des trocknenden Gases erforderliche Energie auf ein Minimum herabsetzt, wodurch der thermische Wirkungsgrad der Vorrichtung beim Trocknen der Platten auf ein Maximum heraufgesetzt wird, wobei in die Vorrichtung zum Regeln eine Vorrichtung zur Messung der Lufttemperatur den Platten vorgeschaltet (86) und nachgeschaltet (88) ist, um die Temperatur im Inneren der Trocknungskammer zu regeln.

2. Vorrichtung nach Anspruch 1, bei welcher die Verbrennungskammer einen Feuerraum (78) in der Verbrennungskammer (21) aufweist, wobei in den Feuerraum (78) ein Kasten (100) einbezogen ist, der über entfernbare Einsätze (102, 106) verfügt.

3. Vorrichtung nach Anspruch 2, bei welcher die entfernbaren Einsätze (102, 106) so konfiguriert sind, dass sie kommunizierende Kammern schaffen, wobei die Kammern die heiße, trockene Luft zu 2 Auslassöffnungen (61, 64) in der Nähe der Wandungen des Gehäuses (10) kanalisieren, wobei die Austrittsöffnungen voneinander beabstandet sind.

4. Vorrichtung nach Anspruch 2, bei welcher die entfernbaren Einsätze (102, 106) außerdem ein Zwischenstück (104) aufweisen, wobei das Zwischenstück (104) und die Einsätze (102, 106) von dem Feuerraumkasten (100) isoliert sind (62).

5. Vorrichtung nach Anspruch 2, bei welcher der Feuerraum (78) einen Flammenstab (108) mit einem Quarzrohr (110) aufweist, das sich um den Flammenstab (108) über dessen größeren Längenabschnitt herum erstreckt.

6. Vorrichtung nach Anspruch 2, bei welcher der Sauerstoff-Messfühler (112) mit dem Feuerraum (78) in Verbindung steht.

7. Vorrichtung nach Anspruch 1, bei welcher die Wasserschleier-Vorrichtung einen Schleier aus Wasser gewährt, das in entgegengesetzter Richtung zur Strömung der Luft strömt, und in die mindestens ein Bett (24, 29) einbezogen ist, das unterhalb der Platten in dem Gehäuse (10) in einem Winkel angeordnet ist, um eine Schwerkraftzuführung des Wassers zu gewähren, wobei das Bett über Rippen (34, 36) darauf verfügt, die das Wasser in separate Bänder (35) davon lenken.

8. Vorrichtung nach Anspruch 7, bei welcher das Wasser entlang eines oberen Teils des Bettes mit Hilfe eines Sammelrohres (26, 30) eingeführt wird, das über eine Vielzahl von Bohrungen darin verfügt, die mit einem aufrecht stehenden Steg (42, 43) in Verbindung stehen, so dass das Wasser glatt auf das Bett ohne zu spritzen abläuft.

9. Vorrichtung nach Anspruch 7, bei welcher das Bett in einer Rückhaltewand (31, 40) endet und Schlitze (51) in den Rippen (34, 36) vorgesehen sind, um dem Wasser den Austritt aus dem Bett und den Bahnen (35) zu ermöglichen.

10. Vorrichtung nach Anspruch 7, bei welcher das Wasser in eine Mulde (58) abläuft und ein Temperaturmessfühler (90) in dieser Mulde angeordnet ist, um die Temperatur des aus der Mulde (58) austretenden Wassers zu messen.

11. Vorrichtung nach Anspruch 1, bei welcher die Blasvorrichtung (17) Gebläse aufweist, die auf einer Welle befestigt sind, wobei die Welle von Lagern (79) gehalten wird, die außerhalb des Gehäuses angebracht sind.

12. Vorrichtung nach Anspruch 1, bei welcher die Blasvorrichtung (17) mindestens ein Gebläse aufweist, das auf einer Achse befestigt ist, die hinter dem Heißgas angeordnet ist, das die Verbrennungskammer verlässt, und bei welcher ein Schacht (89) vorgesehen ist, der hinter der Achse des Gebläses angeordnet ist, wobei der Schacht (89) an seinem unteren Ende eine eingeschränkte Öffnung (118) hat, die so angeordnet ist, dass sie zur Hinterseite des Gehäuses abgewandt von dem Austritt des Heißgases aus der Verbrennungskammer mündet.

13. Vorrichtung nach Anspruch 12, bei welcher ein Temperaturmessfühler (116) an der Oberseite des Schachtes (89) außerhalb des Gehäuses (10) vorgesehen ist.

14. Vorrichtung nach Anspruch 12, bei welcher im Inneren des Schachtes (89) ein Hohlrohr (115) angeordnet ist, dessen eine Ende in näherungsweise der Ebene der Achse (79) der Blasvorrichtung (17) mit der Vorrichtung in Verbindung steht und dessen anderes Ende durch das äußere Ende des Schachtes (89), sowie ein Sauerstoffmessfühler (114), der, auf dem einen Ende des Hohlrohres (115) gegenüber dem Ende außerhalb des Gehäuses (10) befestigt ist.

15. Vorrichtung nach Anspruch 1, bei welcher das Mittel zum Halten der zu trocknenden Akkumulatorplatten mindestens einen Korb (14) mit einem Rand (120) aufweist, auf dem einstellbar bewegliche Gestelle (120) so angeordnet sind, dass sie die Platten halten.

16. Vorrichtung nach Anspruch 15, bei welcher die Gestelle (122) gewellte Oberflächen (124) haben.

17. Vorrichtung nach Anspruch 15, bei welcher die Körbe (14) Griffe (126) daran haben, die daran befestigt Stäbe mit umgekehrtem "V"-Profil aufweisen; sowie Entnahmevorrichtungen (128, 130, 132), die vorgesehen sind, um in die "V"-förmigen Griffe zum Absenken des Korbes in das Gehäuse oder Entfernen des Korbes aus dem Gehäuse einzugreifen.

18. Vorrichtung nach Anspruch 17, bei welcher die Entnahmevorrichtung zum Absenken oder Entfernen des Korbes einen Stab (128) mit mindestens einem Haken (130, 132) daran aufweist, wobei der Stab so angeordnet und bemessen ist, dass er zwischen die Innenwandung des Gehäuses und die Außenwandung des Korbes passt, so dass nachdem der Stab darin eingesetzt und sodann gedreht wird, bei Entfernung der Entnahmevorrichtung in den "V"-förmigen Abschnitt des Griffes (126) eingreift.

19. Vorrichtung nach Anspruch 18, bei welcher eine Vielzahl von Körben in der Vorrichtung verwendet wird und die Haken (103, 132) an der Entnahmevorrichtung um einen größeren vertikalen Abstand voneinander beabstandet sind, als der vertikale Abstand der "V"-förmigen Griffe (126), wenn die Körbe übereinander gestapelt werden, so dass, wenn die Stäbe (128) gedreht und herausgezogen werden, ein oberer Haken (130) in den oberen "V"-förmigen Abschnitt eines oberen Korbgriffes eingreift, bevor der untere Haken (132) des "V"-förmigen Abschnittes des unteren Korbgriffes eingreift.

20. Vorrichtung nach Anspruch 1, bei welcher die Vorrichtung mit einer Türvorrichtung zum Öffnen in das Gehäuse ausgestattet ist, um so den Körben zu ermöglichen, in die Kammer abgesenkt zu werden, sowie zum Schließen, um der Vorrichtung das Arbeiten im Trocknungsprozess zu ermöglichen, wobei die Türvorrichtung über eine Tür verfügt, die an ihrer einen Seite eingelenkt ist und eine oder mehrere Kolben- und Zylinderanordnungen hat, die an der Tür und an dem Gehäuse befestigt sind, um die Tür zu betätigen.

21. Vorrichtung nach Anspruch 20, bei welcher die Türvorrichtung eine Tür (12) mit einer Dichtung um ihre Kante herum versehen ist, die mit dem Gehäuse zusammenpasst, um einen Sauerstoffaustritt während der Betriebsfunktion der Vorrichtung zu vermeiden.

22. Verfahren zum Trocknen geladener Akkumulatorplatten, umfassend die Schritte:
die geladenen Platten in eine Vorrichtung legen, die eine Trockenkammer (16) aufweist; Bereitstellen eines Stroms eines im Wesentlichen von Sauerstoff freien trocknenden Gases mit relativ geringer Feuchtigkeit, wobei der Strom so gelenkt wird, dass er über die Platten strömt, um deren Trocknung zu bewirken; Kondensieren des Wassers aus dem Gas, das über die Platten zu deren Trocknung geströmt ist; welches Verfahren **gekennzeichnet ist durch** die Schritte:
dieses Gas über die Oberfläche eines Wasserschleiers strömen lassen, der in Gegenrichtung zu dem Gas fließt, ohne Wassertröpfchen in das Gas einzuführen; und
Aufrechterhalten der Temperaturdifferenz innerhalb der Trockenkammer derart, dass diese Wärme hauptsächlich zum Trocknen der Platten verwendet wird und nur minimal zum Wiedererhitzen der Luft aus dem Wärmeverlust in Folge des Kondensationsprozesses des Verfahrens, indem die Temperatur des trocknenden Gases gemessen wird (86), bevor es über die Platten strömt; Messen (88) der Temperatur des trocknenden Gases, nachdem es über die Platten geströmt ist; Messen (90) der Temperatur des aus der Vorrichtung austretenden Wassers; sowie Regeln der Temperatur und der Strömungsgeschwindigkeit des Wasserschleiers entsprechend diesen Messungen.

23. Verfahren nach Anspruch 22, bei welchem die Temperatur des austretenden Wassers im Bereich von 46 bis 49°C (115° bis 120°F) und am meisten bevorzugt 46°C (115°F) aufrecht erhalten wird.

24. Verfahren nach Anspruch 23, bei welchem der Gasstrom über der Oberfläche des Wasserschleiers so geregelt wird, dass er unterhalb der Geschwindigkeit ist, die "Whitecaps" hervorrufen würde.

25. Verfahren nach Anspruch 22, bei welchem das thermische Instabilwerden in der Vorrichtung vermieden wird, indem die Temperatur des Heißgases in der Gebläsekammer gemessen (116) wird, indem das Gas durch eine gedrosselte Öffnung (118) in der Nähe der Achse der Gebläse (17) in dem Aufbau geführt wird und die Temperatur außerhalb der Vorrichtung abgelesen wird.

26. Verfahren nach Anspruch 22, bei welchem das trocknende Gas in einem begrenzten Bereich erhitzt und der Sauerstoffgehalt in diesem Gas in dem begrenzten Bereich gemessen wird und das trocknende Gas aus diesem begrenzten Bereich austritt.

27. Verfahren nach Anspruch 22, bei welchem die Methode des Erhitzens und Trocknens der Platten das einschließen der Platten in einem geschlossenen Bereich (10) umfasst, aus dem zuerst die brennbaren Gase ausgespült worden sind, und Erhitzen der Luft in dem geschlossenen Bereich, bis die Temperatur mehr als 82°C (180°F) erreicht, und sodann Einführen des Wasserschleiers.

28. Vorrichtung nach Anspruch 1, bei welchem der Wasserschleier in Gegenrichtung zu dem aus den Platten austretenden Gas strömt.

29. Vorrichtung nach Anspruch 1, bei welchem eine Vielzahl von Wasserschleiern vorgesehen ist, um mit dem aus den Platten austretenden Gas in Kontakt gebracht zu werden.

## Revendications

1. Appareil destiné à sécher des plaques de batterie chargées possédant un boîtier (10) pouvant maintenir intérieurement une pression de gaz positive, une chambre de séchage (16) disposée à l'intérieur dudit boîtier et ayant un moyen (14) servant à soutenir des plaques de batterie devant être séchées dans une position telle que du gaz peut se déplacer sur les plaques, une chambre de combustion (21) disposée à l'intérieur dudit boîtier et servant à fournir un gaz sec et chaud, sensiblement sans oxygène, à un moyen de soufflerie (17) qui souffle le gaz sur lesdites plaques afin d'effectuer le séchage des plaques en éliminant l'humidité de celles-ci, ledit appareil étant **caractérisé par** :
un moyen (24, 26, 29, 30, 34, 36) de formation de nappe d'eau permettant de produire une nappe d'eau de refroidissement en écoulement de manière qu'elle soit en contact avec le gaz quittant lesdites plaques et qu'elle condense l'humidité retirée desdites plaques pendant le séchage ; et
un moyen de commande de température servant à maintenir une certaine différence de température avec ladite chambre de séchage, ledit moyen de commande de température minimisant la chaleur utilisée pour compenser les pertes de chaleur dues à ladite condensation de l'humidité du gaz de séchage, de façon à minimiser l'énergie nécessaire pour élever la température du gaz de séchage, et ainsi maximiser le rendement thermique dudit appareil lors du séchage des plaques, le moyen de commande comportant des moyens (86 et 88) de mesure de la température de l'air respectivement en amont et en aval des plaques afin de commander la température régnant à l'intérieur de ladite chambre de séchage.

2. Appareil selon la revendication 1, où la chambre de combustion comprend un foyer (78) dans la chambre de combustion (21), ledit foyer (78) comportant un carter (100) qui possède des éléments rapportés (102, 106) qui peuvent enlevés.

3. Appareil selon la revendication 2, où les éléments rapportés (102, 106) pouvant être enlevés sont configurés de façon à produire des chambres communicantes, lesdites chambres canalisant l'air sec et chaud jusqu'à deux orifices d'évacuation (61, 64) proches des parois dudit boîtier (10), lesdits orifices d'évacuation étant écartés l'un de l'autre.

4. Appareil selon la revendication 2, où les éléments rapportés (102, 106) pouvant être enlevés comprennent également un élément d'écartement (104), ledit élément d'écartement (104) et lesdits éléments rapportés (102, 106) étant isolés (62) vis-à-vis du carter (100) du foyer.

5. Appareil selon la revendication 2, où le foyer (78) possède une tige de foyer (108) ayant un tube de quartz (110) qui se prolonge autour de ladite tige de foyer (108) sur la plus grande partie de la longueur de celle-ci.

6. Appareil selon la revendication 2, où un détecteur d'oxygène (112) communique avec ledit foyer (78).

7. Appareil selon la revendication 1, où le moyen de formation de nappe d'eau produit une nappe d'eau qui s'écoule dans le sens opposé à celui de l'écoulement de l'air et qui comporte au moins une plate-forme (24, 29) placée au-dessous desdites plaques dans ledit boîtier (10) suivant un angle propre à assurer un écoulement de l'eau par gravité; ladite plate-forme ayant des ailettes (34, 36) qui dirigent l'eau dans des nervures séparées (35) de celui-ci.

8. Appareil selon la revendication 7, où de l'eau est introduite le long d'une partie supérieure de ladite plate-forme par un tuyau de tête (26, 30) possédant une pluralité de trous qui communiquent avec une nervure dressée verticalement (42, 43), de façon que l'eau courre régulièrement sur ladite plate-forme sans éclabousser.

9. Appareil selon la revendication 7, où ladite plate-forme se termine par une paroi de retenue (31, 40) et des fentes (51) sont ménagées dans lesdites ailettes (34, 36) afin de permettre à l'eau de quitter ladite plate-forme et lesdites nervures (35).

10. Appareil selon la revendication 7, où l'eau s'évacue dans une gouttière (58) et un capteur de température (90) est placé dans ladite gouttière afin de mesurer la température de l'eau sortant de ladite gouttière (58).

11. Appareil selon la revendication 1, où ledit moyen de soufflerie (17) comprend des ventilateurs montés sur un arbre, ledit arbre étant porté par des paliers (79) montés à l'extérieur du boîtier.

12. Appareil selon la revendication 1, où ledit moyen de soufflerie (17) comprend au moins un ventilateur monté sur un axe positionné en aval du gaz chaud quittant la chambre de combustion, et une cheminée (89) est placée en une position postérieure à l'axe du ventilateur, ladite cheminée (89) ayant une ouverture limitée (118) à son extrémité inférieure, qui est positionnée pour s'ouvrir sur l'arrière du boîtier à distance du gaz chaud sortant de la chambre de combustion.

13. Appareil selon la revendication 12, où un capteur de température (116) est placé à la partie supérieure de ladite cheminée (89) à l'extérieur dudit boîtier (10).

14. Appareil selon la revendication 12, où un tube creux (115) est placé à l'intérieur de ladite cheminée (89), qui possède une extrémité communiquant avec ledit appareil approximativement au niveau du plan de l'axe (79) du moyen de soufflerie (17) et une autre extrémité communiquant par l'intermédiaire de l'extrémité externe de ladite cheminée (89), et un détecteur d'oxygène (114) est monté sur ladite extrémité, citée en premier, du tube creux (115) à l'opposé de l'extrémité extérieure audit boîtier (10).

15. Appareil selon la revendication 1, où le moyen servant soutenir les plaques de batterie devant être séchées comprend au moins un panier (14) ayant un rebord (120) sur lequel des râteliers (122) mobiles de façon réglable sont positionnés de façon à retenir lesdites plaques.

16. Appareil selon la revendication 15, où lesdits râteliers (122) présentent des surfaces supérieures striées (124).

17. Appareil selon la revendication 15, où lesdits paniers (14) ont des poignées (126) comprenant des tiges en forme de "V" retournés qui leur sont fixées ; et des moyens d'enlèvement (128, 130, 132) sont prévus de façon à venir en prise avec lesdites poignées en forme de "V" afin d'abaisser ledit panier dans ledit boîtier ou de retirer ledit panier dudit boîtier.

18. Appareil selon la revendication 17, où ledit moyen d'enlèvement servant à abaisser ou enlever le panier comprend une tige (128) possédant au moins un crochet (130, 132), ladite tige étant placée et dimensionnée de façon à s'ajuster entre la paroi interne dudit boîtier et la paroi externe dudit panier, de façon que, après qu'on y a inséré la tige et qu'on l'a ensuite fait tourner, au moment de l'enlèvement, ledit moyen d'enlèvement vient en prise avec ladite partie en forme de "V' de ladite poignée (126).

19. Appareil selon la revendication 18, où on utilise une pluralité de paniers dans ledit appareil, et les crochets (103, 132) se trouvant sur ledit moyen d'enlèvement sont écartés les uns des autres d'une distance verticale supérieure à l'écartement vertical des poignées en forme de "V" (126) lorsque lesdits paniers sont empilés les uns sur les autres, de sorte que, lorsqu'on fait tourner lesdites tiges (128) et qu'on les enlève, un crochet supérieur (130) vient en prise avec la partie en forme de 'V" supérieure de la poignée d'un panier supérieur avant que le crochet inférieur (132) ne vienne en prise avec la partie en forme de "V" de la poignée du panier inférieur.

20. Appareil selon la revendication 1, où l'appareil est dote d'un moyen formant une porte servant à ouvrir dans ledit boîtier de façon à permettre que des paniers soient abaissés jusque dans ladite chambre, et permettant de fermer pour permettre que ledit appareil fonctionne dans le processus de séchage, ledit moyen porte possédant une porte articulée suivant un de ses bords et ayant un ou plusieurs agencements piston-cylindre fixés à ladite porte et audit boîtier afin d'actionner ladite porte.

21. Appareil selon al revendication 20, où ledit moyen porte possède une porte (12) dotée d'un joint étanche autour de son bord en correspondance avec ledit boîtier, de façon à empêcher que l'oxygène ne fuit à l'intérieur pendant le traitement effectué par ledit appareil.

22. Procédé de séchage de plaques de batterie chargées, comprenant les opérations suivantes :
placer les plaques chargées dans un appareil comprenant une chambre de séchage (16) ;
fournir un écoulement de gaz de séchage sensiblement dépourvu d'oxygène présentant une humidité relativement basse et dirigé de façon qu'il passe sur lesdites plaques afin de les sécher ;
faire se condenser l'eau présente dans le gaz qui est passé sur les plaques pour les sécher,
ledit procédé étant **caractérisé par** les opérations suivantes :
faire passer ce gaz sur la surface d'une nappe d'eau s'écoulant dans un sens opposé à celui du gaz, sans introduire de gouttelettes d'eau dans le gaz ; et
maintenir la différence de température régnant à l'intérieur de ladite chambre de séchage de façon que la chaleur soit utilisée principalement pour sécher les plaques et, de façon minimale, pour réchauffer l'air relativement à la chaleur perdue du fait du processus de condensation effectuée dans ledit procédé, en mesurant (86) la température du gaz de séchage avant qu'il ne passe sur lesdites plaques, en mesurant (88) la température du gaz de séchage après qu'il a passé sur lesdites plaques ; en mesurant (90) la température de l'eau sortant dudit appareil ; et en régulant la température et le débit de ladite nappe d'eau en fonction de ces mesures.

23. Procédé selon la revendication 22, où la température de l'eau qui sort est maintenue dans l'intervalle de 46° à 49°C (115° à 120°F) et, de manière préférée, à 46°C (115°F).

24. Procédé selon la revendication 23, où l'écoulement de gaz sur la surface de la nappe d'eau est régulé de façon qu'il soit en deçà du débit qui provoquerait des "moutons".

25. Procédé selon la revendication 22, où on empêche l'emballement thermique de ladite machine en mesurant (116) la température du gaz chaud dans la chambre de soufflerie en faisant passer ce gaz dans une ouverture limitée (118) proche de l'axe des ventilateurs (17) présents dans la machinerie et en lisant la température à l'intérieur de l'appareil.

26. Procédé selon la revendication 22, où ledit gaz de séchage est chauffé dans une zone confinée et la teneur en oxygène dudit gaz est mesurée dans ladite zone confinée et au sortir de ladite zone confinée.

27. Procédé selon la revendication 22, où le procédé de chauffage et de séchage de plaques comprend le confinement des plaques dans une zone fermée (10) qui a d'abord été purgée des gaz combustibles et le chauffage de l'air se trouvant dans ladite zone fermée jusqu'à ce que la température atteigne une valeur supérieure à 82°C (180°F), après quoi on introduit ladite nappe d'eau.

28. Appareil selon la revendication 1, où la nappe d'eau s'écoule dans un sens opposé à celui du gaz quittant lesdites plaques.

29. Appareil selon la revendication 1, où il est prévu une pluralité de nappes d'eau destinées à venir en contact avec ledit gaz qui quitte lesdites plaques.
